

May 14, 1946.

G. F. WOMBLE

2,400,327

SELVAGE FOR RAYON FABRICS

Filed Aug. 2, 1944

*Fig. 1*



*Fig. 2*



*Fig. 3*



*Fig. 4*



← SELVAGE → FABRIC →



Inventor

**GLENN F. WOMBLE**

By *Worley L. Parrott*

Attorney

## UNITED STATES PATENT OFFICE

2,400,327

## SELVAGE FOR RAYON FABRICS

Glenn F. Womble, Danville, Va., assignor to  
Riverside & Dan River Cotton Mills, Incorporated, a corporation of Virginia

Application August 2, 1944, Serial No. 547,815

3 Claims. (Cl. 139—426)

In the wet processing of rayon fabrics, such as for example, the usual dyeing or finishing treatments applied to such fabrics, there is encountered the problem of tearing of the fabric because of its inherent weakness when wet. It is particularly characteristic of the rayon fabrics, as contrasted with the fabrics of natural fibers, such as cotton, linen and wool, to decrease substantially in tensile strength when these rayon fibers or filaments are wet. And when the wet rayon fabrics are subjected to tension or other stresses in processing such as the conventional boiling out and dyeing operations on a jig and in finishing operations carried out on the open width of the fabric, there is a common tendency for the rayon fabric to tear. The tear usually begins at the selvage edge, and once the break or tear has started in the fabric it will continue even more easily and result in a damaged product. Oftentimes this necessitates shutting down the manufacturing operation, thereby losing valuable time and expensive chemicals, until the torn fabric can be mended.

This problem applies especially to operations in which the rayon fabric is processed in the open width and is moving very rapidly through processing machinery where dyes or other wet treatments are applied to the fabric and the fabric is at that time subjected to strains or stresses.

In accordance with my present invention, I have discovered a simple but expedient means for overcoming this problem that has proven very bothersome in the commercial processing of rayon fabrics. I have found that if some of the rayon threads, commonly called "ends," in the selvage edge of the rayon fabric are substituted by cotton threads, even though of similar size, the strength of the selvage edge is markedly increased and thereby effectively prevents tearing of the selvage edge and the rayon fabric during the wet processing treatment. In this selvage construction I have put into practical use the property of the cotton threads of not weakening when wet and, on the contrary, of actually becoming stronger when wet than when dry. When rayon is wet with water it loses about half of its dry strength. In contradistinction, cotton when wet with water substantially increases in strength, such as for example 15% in a typical case. Furthermore, if it is so desired, all of the rayon threads in the selvage edge may be substituted by the cotton threads or fibers; or blends or twists of rayon and cotton threads or fibers may be used. In actual commercial practice, a substitution of about 15% to 30% of the rayon threads by

cotton threads in the selvage has given very satisfactory results.

Different forms of fabric embodying my invention and in the construction and use of which the objects herein set out, as well as others, may be attained, are illustrated in the accompanying drawing, in which—

Fig. 1 is a face view of a piece of fabric embodying my invention.

Fig. 2 is an end view of the fabric shown in Fig. 1.

Figs. 3 and 4 are end views showing different forms of the invention.

In each of the several figures of the drawing a rayon fabric 10 is shown having a selvage edge 11 in which certain of the rayon threads have been replaced by cotton threads 12, other rayon warp threads being shown at 13 and weft threads at 14. These figures are merely illustrative of various forms of selvage arrangement embodying the present invention.

In an illustrative but non-limiting example of a rayon fabric, the selvage edge will contain from about 12 to 24 warp threads; and these warp threads are usually of two-ply yarn. In a typical, specific case of this type, I have substituted 4 of the warp ends, normally rayon threads, by 4 cotton warp threads and have so increased the strength of the selvage that the problem of tearing when wet is substantially completely eliminated. In other illustrative commercial examples, the number of cotton warp ends may be reduced to two ends, and, on the other hand, may be increased to 6 or 8 cotton warp ends, or, as above suggested, may replace the entire 12 to 24 warp ends or rayon threads normally used in the selvage, as varying processing conditions may require.

For a further and more detailed understanding of my present invention, the following illustrative but non-limiting example of the adaptation of my improvement to a commercial operation is given.

A viscose rayon fabric is woven in the conventional manner except the selvage is inlaid with 4 ends of two-ply cotton yarn replacing four of the 24 ends of two-ply viscose yarn in the selvage. In this specific combination the cotton ends and the viscose ends are so blended that they are substantially indistinguishable in the selvage edge and the selvage appears to be exactly the same as though all viscose yarn were used.

Now this rayon fabric with the viscose-cotton warp selvage is desized, boiled out, and prepared for dyeing in open width on a jigger, and then dried on a frame and dyed on a continuous dyeing

machine such as normally used in the continuous dyeing of cotton fabrics with vat colors. In these operations the fabric is subjected to considerable tensile stresses and is very subject to tearing or breaking if the selvage is not reinforced properly as is done in my invention.

The term "rayon" as used herein is used in a generic sense to identify broadly the substitute silks which have the above described tendency of weakening and tearing when wet. These substitute silks include the so-called acetate silks which consist of acetic esters of cellulose; and the cuprammonium, nitrocellulose and viscose rayon silks which belong to the class of regenerated cellulose products, the most common commercial example of which is viscose rayon; and the other synthetic fibers or filaments that weaken when wet; or are inherently weak.

Instead of using cotton threads for the strengthening elements in the selvage edge as described above, other similar and suitable threads or fibers may be used, including linen, jute, hemp, ramie; and some of the synthetic fibers which do not weaken when wet, such as "Saran" and

"Vinyon." These natural and synthetic fibers are defined generically in the claims herein as "reinforcing fiber."

Various modifications and changes may be made in the above described materials, constructions and processes without departing from the scope of my invention, some of the novel features of which are defined in the appended claims.

I claim:

- 10 1. A textile fabric having a body portion composed of warp and weft threads of conventional rayon as defined herein, which have a tendency to become weakened when they are wet, and a selvage edge including at least two and not more than twenty-four warp threads of a reinforcing fiber that does not become weakened when it is wet and serves to strengthen said textile fabric during wet processing.
- 15 2. A textile fabric according to claim 1 in which the reinforcing fiber is a natural cellulose fiber.
- 20 3. A textile fabric according to claim 1 in which the reinforcing fiber is cotton.

GLENN F. WOMBLE.